

## 1

3,487,593

METHOD FOR PRODUCING A STRETCH-  
RESISTANT COATED ABRASIVE PRODUCTDaniel R. Vinard, Le Vesinet, France, assignor to  
Norton Company, Worcester, Mass., a corporation  
of MassachusettsNo Drawing. Filed Aug. 29, 1967, Ser. No. 663,985  
Claims priority, application France, Oct. 31, 1966,

82,306

Int. Cl. B24d 11/02

U.S. CL. 51—293

## 1 Claim

## ABSTRACT OF THE DISCLOSURE

The use of a tightly woven cloth backing containing polynotic threads as the warp or fill threads of the cloth in an amount sufficient to reduce the stretch of the finished coated abrasive article by at least 25% in the direction in which the polynotic threads extend.

The present present invention has general reference to coated abrasive products and more particularly relates to the backings suitable for the manufacture of coated abrasive products.

It is known in certain industries to use so-called "polynotic threads" which consist of filaments made of regenerated cellulose, the chains of which have an orientated structure and a high molecular weight, and which may be obtained by the viscose process, the latter being suitably modified.

It is known that polynotic threads have a very orientated structure, a high breaking strength and a high modulus of elasticity. Owing particularly to their breaking strength, they have been utilized according to the former technique, as a reinforcement or armature for applications including a coating constituted by rubber or equivalent material, the threads being imbedded in the product. Conveyor belts and tires, for example, have been manufactured with such polynotic threads.

The researches which have lead to the invention have revealed that it is possible to make use in new fashion of the characteristics of polynotic threads corresponding to a high modulus of elasticity for manufacturing backings for coated abrasive products, every time it is desired to obtain for the manufactured product a specific elongation of small value. As a matter of fact, it is known that the coated abrasive products, particularly those which are utilized in belt form must be capable of lending themselves to an elongation of small value in one direction which corresponds to the direction in which the stresses are exerted during the abrasion work.

Moreover, researches have shown that the polynotic threads have a good property of absorbing aqueous suspensions, a characteristic which remained unemployed in the case of a coating made with a rubber mass.

The invention makes use of these characteristics, and is materialized in a backing for coated abrasive products constituted by a woven backing in which the weft threads or the warp threads of the cloth are constituted at least partly by polynotic threads.

The warp or the weft of said cloth (as the case may be) may be constituted by usual cotton, which is the material generally utilized for the manufacture of the known woven backings.

According to a feature of the invention, the texture of the woven backing including polynotic threads as warp threads or weft threads should be as tight as possible for staving off sliding or distortion of the cloth, and the weave is suitably constituted by a "cotton serge"

## 2

or "satin" weave so as to increase the resistance to distortion and the compactness of the cloth. The weight of the threads in the chosen direction is at least equal to 60 g./sq. meter and the total weight of the cloth is preferably equal to or higher than 200 g./sq. meter. This characteristic is in opposition to that presented by the textures of known reinforcements constituted by polynotic threads (or containing such threads) which, as a rule are very loose so as to permit the cloth to become distorted and elongated. As a matter of fact, in the known textures, the polynotic threads are provided only to enhance the mechanical resistance of the reinforcement owing to their breaking strength. In the case of the new application which is the object of the invention, the characteristic of small elongation presented by the polynotic threads is utilized in the desired direction while taking into consideration the work which is envisaged for the product.

Of course, these polynotic threads may, as aforesaid, constitute the whole weft or only a part thereof, or alternatively the whole warp or only a part thereof, according to the desired characteristics. However, it could be possible, without departing from the scope of the invention, to manufacture a backing for coated abrasive products, in which both the weft and the warp would be constituted wholly or partly by polynotic threads, although normally this dual utilization does not meet the conditions of resistance to elongation in one single direction which are to be obtained for a satisfactory backing for coated abrasive products utilized in band form.

30 The utilization of polynotic threads for the manufacture of woven backings for coated abrasive products advantageously facilitates the coating operation according to the finishing methods which are generally utilized for the backings made of woven cotton, according to which animal glues, starch paste, etc., are utilized. The researches which have led to the invention have shown, as previously indicated, that these polynotic threads have a good property of absorption for aqueous suspensions. This characteristic is necessary for realizing coated abrasive products, in order to ensure retention of the abrasive grains.

35 The invention also includes, as new articles of manufacture, the coated abrasive products, particularly in the form of belts, comprising a woven backing, the warp or the weft of which is constituted at least partly by polynotic threads.

40 The way of manufacturing a woven backing according to the invention and a coated abrasive product comprising such a backing including polynotic threads are indicated hereafter by way of non-limitative example.

## EXAMPLE

45 The unbleached material utilized for constituting the backing according to the invention is a  $\frac{1}{4}$  satin including a cotton warp made of 38 threads Nm. 28 and a weft made of polynotic threads including 21 threads Nm. 10, 7. Such a backing may be woven in conventional fashion.

50 The backing being thus constituted, the coating utilized for the manufacture of the abrasive product is performed according to the finishing methods generally utilized for the cloths made of 100% cotton. After finishing is effected, the maximum elongation at rupture of the finished cloth in the direction of the weft is reduced by about 25% with respect to that obtained with a cloth made of natural cotton.

55 The coating of the abrasive grains may then be performed by means of usual phenolic binders. It has been stated that the maximum elongation at rupture of the coated abrasive product, which is thus obtained, while measured in the direction of the weft, is reduced by nearly 50% with respect to that which is obtained with a usual cloth made of natural cotton.

The results which are obtained, as far as the reduction of elongation at rupture is concerned, are clearly shown by comparative tests made with an unbleached material, as aforesaid, utilized according to the invention and with an unbleached material made of 100% cotton, while measuring the elongation at rupture in the direction of the weft. The weight of each unbleached material is about 350 g./sq. meter. These results are indicated in the following table:

|                              | 10                                      | 10             | 10 | 10 |
|------------------------------|-----------------------------------------|----------------|----|----|
|                              | Welt<br>made of<br>polynotic<br>threads | 100%<br>cotton |    |    |
| Finished cloth, percent..... | 17                                      | 22.5           | 15 |    |
| Coated product, percent..... | 14.5                                    | 26             |    |    |

(Silicon carbide, grain No. 50 and phenolic binders)

The coated product may be particularly utilized in the form of "sectional belts," the sections being cut out in a direction defining an angle smaller than 45°, with the direction of the weft of the cloth constituting the backing.

Tests have shown that the elongation of the coated abrasive products manufactured with said belts is quite small.

The embodiment of the invention as described may

be varied in the field of technical equivalencies without departing from the scope of the invention.

I claim:

5 1. In a method for producing a coated abrasive product having reduced stretch in at least one direction, wherein said coated abrasive product consists of abrasive grains adhesively bonded to a flexible backing, the improvement which comprises:

- (a) providing a woven backing for said coated abrasive product containing a plurality of polynotic threads having a weight of at least 60 g./m.<sup>2</sup> extending in at least one direction; and
- (b) weaving said threads in a satin weave pattern into said woven backing in a tight, closely-packed relationship to minimize sliding and distortion of said backing.

#### References Cited

##### UNITED STATES PATENTS

- |           |         |               |       |          |
|-----------|---------|---------------|-------|----------|
| 2,284,738 | 6/1942  | Hurst         | ----- | 51—303   |
| 2,397,808 | 4/1946  | Riding        | ----- | 51—303   |
| 2,817,371 | 12/1957 | Bussiere      | ----- | 51—298.1 |
| 3,419,652 | 12/1968 | Kubota et al. | ----- | 264—189  |

20 25 DONALD J. ARNOLD, Primary Examiner

51—298, 303

U.S. Cl. X.R.